

[72] Inventor **Jacques A. DeCuyper**  
 Sterrebeek, Belgium  
 [21] Appl. No. **868,241**  
 [22] Filed **Oct. 21, 1969**  
 [45] Patented **Mar. 30, 1971**  
 [73] Assignee **Societe De Produits Chimiques D'Auby**  
 Neuilly-sur-Seine (Hauts de Seine), France  
 [32] Priority **May 11, 1966**  
 France  
 [33] **61,081**  
 Continuation of application Ser. No.  
 637,621, May 11, 1967, now abandoned.

[54] **METHOD FOR THE FLOTATION OF OXIDIC ORES  
 WITH CALCAREOUS AND DOLOMITIC GANGUE**  
 7 Claims, No Drawings  
 [52] U.S. Cl..... **209/166**  
 [51] Int. Cl..... **B03d 1/02**  
 [50] Field of Search..... **209/166,  
 167; 210/54**

[56] **References Cited**  
 UNITED STATES PATENTS  
 1,312,668 8/1919 Bacon ..... 209/167X  
 2,740,522 4/1956 Aimone ..... 209/166  
 2,955,932 10/1960 Goren ..... 210/54X  
 2,980,609 4/1961 Mouse ..... 210/54  
 FOREIGN PATENTS  
 141,827 11/1960 U.S.S.R. ..... 209/167  
 378,063 7/1932 Great Britain ..... 209/167  
*Primary Examiner*—Frank W. Lutter  
*Assistant Examiner*—Robert Halper  
*Attorney*—Stevens, Davis, Miller & Mosher

**ABSTRACT:** A method for the flotation of minerals and ores with a calcareous and dolomitic gangue, such as oxidized ores, especially of copper, in which there are incorporated in the flotation pulps, when so required, together with modifying reagents acting on the minerals to be collected, modifying products acting on the gangues, especially on calcareous and dolomitic gangues, the said gangue-modifying products being preferably agents selected from the group comprising the polymers of acrylic acid, their derivatives and their equivalents which are soluble in water.

**METHOD FOR THE FLOTATION OF OXIDIC ORES WITH CALCAREOUS AND DOLOMitic GANGUE**

This application is a continuation of application Ser. No. 637,621, filed 5/1967 and now abandoned.

In the flotation of minerals, and especially of ores, it is always sought to improve the selectivity of the separation between the minerals which it is desired to recover and those of the gangue. To this end, use is frequently made of reagents known as modifiers, the effect of which is to cause a segregation of the minerals from the gangue, so as to prevent them from floating with the minerals to be collected. Amongst the reagents currently used for this purpose, there must be cited the alkalis such as sodium carbonate, lime and caustic soda, sodium silicate, acids, sodium cyanide and sulfides, etc.

These reagents are however not sufficient in very many cases, and especially in the case of oxidized ores and when the gangues are calcareous and dolomitic, the selectivity then frequently leaving much to be desired, because the reactions of the rich minerals and those of the minerals of the gangue are not sufficiently differentiated.

In order to overcome this difficulty, it is proposed, in accordance with the invention, to incorporate in the flotation pulps, when so desired at the same time with modifying reagents acting on the minerals to be collected, modifying reagents acting on the gangues, especially on the calcareous and dolomitic gangues.

As modifying reagents of the gangues, there are preferably chosen, in accordance with the invention, agents comprised in the family of the polymers of acrylic acid, of their derivatives and their equivalents which are soluble in water. The solutions of polymers utilized within the framework of the invention have advantageously a mean viscosity (Brookfield) at 25° C. comprised between 5 and 500 centipoises (for an aqueous solution containing 20 percent of active products), the best results being obtained with solutions having a viscosity comprised between 5 and 100 centipoises. Higher viscosities, corresponding to molecular weights in excess of 10,000 have proved to be much less favorable, since they give rise to flocculations which adversely affect the process of flotation employed according to the invention.

The modifying agents according to the invention advantageously correspond to the following general formula (or the like):



in which R represents H or  $\text{CH}_3$ , X represents H or a cation which may be mineral (Na, Li, K,  $\text{NH}_4$ , etc.) or organic (organic bases giving, with the polymers forming the object of the invention, compounds soluble in water),  $n$  being a number which is very variable according to the degree of polymerization, the said degree of polymerization being approximately estimatable as a function of the viscosity of the solutions obtained.

These acrylic polymers correspond advantageously to the criteria of viscosity specified above, and are preferably obtained by polymerization of acrylic acid or methacrylic acid or of their salts, following the known method making use of REDOX catalysts which contain simultaneously an oxidizing agent and a reducing agent, e.g. hydrogen peroxide + ferrous sulfate or ammonium persulfate + sodium bisulfite, etc. The dosing of the catalyst employed, the regulation of the reaction temperatures and the addition of regulators such as methanol,

acetone, or certain metallic ions, make it possible to limit the degree of polymerization to a suitable value.

The achievement of a good selectivity is particularly difficult to the case of oxidized ores, especially when these latter are floated by means of collectors such as fatty acids, alcohols or their derivatives (soaps, sulfonates, sulfates, phosphates, amine salts, etc.) The majority of the common ions ( $\text{Fe}^{+++}$ ,  $\text{Ca}^{++}$ ,  $\text{Mg}^{++}$ ...) which are practically always present in a flotation pulp, have in fact a tendency to "activate" the minerals of the gangue in the presence of these collectors.

Furthermore, when the gangue contains dolomite, the latter is even liable to be collected in preference to the useful minerals. Thus, in the treatment by flotation of oxidized ores of copper, lead and zinc, recourse is frequently had to the method of sulfuration which is known per se.

In accordance with the invention, this sulfuration is effected by addition to the pulp of ground ore, or reagents such as sodium hydrosulfide, or sodium, barium or ammonium sulfides. The oxidized minerals which it is desired to recover in the

foam during the flotation, thus become superficially sulfurized. For this reason, they behave like sulfides, and their separation by flotation is then effected by means of the collector reagents utilized currently in the flotation of sulfurated ores.

The application of the method and the products in accordance with the invention makes it possible to obtain, for the same consumption of collector reagent, a marked increase in the selectivity of separation, without reducing the rate of recovery. This latter rate is even frequently increased, the floatability of the useful material being improved due to the fact that its surface is less coated by the sludges of the gangue. In addition, the method offers the following advantages:

1. It reduces the content of lime and magnesia in the concentrates, thus improving the metallic content of these latter.

2. This results in a reduction of the cost of consumption of acid when the concentrated oxide must be subsequently treated by lixiviation.

3. It improves the flotation of the sludges and increases their rate of recovery.

4. The addition of the modifiers proposed according to the invention does not necessitate any conditioning over a long period and does not have any adverse effect on the stability of the foam.

5. The content of the concentrates being increased for the same recovery of metal, the weight of concentrates to be filtered is reduced. This results in a reduction of the costs of filtration and of the costs of any possible transport of the concentrates.

Other characteristics of the invention will become apparent from the description which follows below of examples of application of the invention. The first examples relate to a retreatment of residues of the flotation of the sulfides of a sulfurated and oxidized mixed copper ore obtained from the Katanga.

In order to permit comparison to be made, the residues in question were first subjected to a standard sulfuration and flotation treatment in a laboratory Denver cell. The consumption of reagents was as follows:

Sulfurating agent: 1.5 kg. of sodium hydrosulfide per ton of ore;

Collector 80 grams of potassium amylxanthate per ton of ore;

Foaming agents: 190 grams of emulsion of pine oil and gasoline per ton of ore.

The results are shown in the following table.

| Product                | Weight percent | Cu percent | Efficiency, Cu percent | CaO+MgO, percent | Efficiency CaO+MgO, percent |
|------------------------|----------------|------------|------------------------|------------------|-----------------------------|
| 1st concentrate.....   | 1.7            | 25.80      | 23.8                   | 5.35             | 0.6                         |
| 2nd concentrate.....   | 1.2            | 19.80      | 12.9                   | 6.21             | 0.5                         |
| 3rd concentrate.....   | 1.0            | 17.65      | 9.3                    | 6.72             | 0.4                         |
| Total concentrate..... | 3.9            | 21.90      | 46.0                   | 5.96             | 1.5                         |
| Waste.....             | 96.1           | 1.05       | 54.0                   | 15.47            | 98.5                        |
| Supply.....            | 100.0          | 1.87       | 100.0                  | 15.10            | 100.0                       |

These results will be compared with those obtained in three examples of application of the method and products according to the invention, which utilize, as indicated below:

1. A modifying agent A according to the above-specified formula and constituted by an aqueous solution with 20 percent of polyacrylic acid having a Brookfield viscosity at 25°C. equal to 40 centipoises.

2. A modifying agent B, similar to the preceding, having a viscosity equal to 50 centipoises.

3. A modifying agent C, having a viscosity equal to 13 centipoises.

In the first example, 250 grams of polymer A were added; in the second, 330 grams of polymer B, and in the third example, 158 grams of polymer C per ton of ore, all the other conditions of the sulfuration treatment being furthermore maintained the same.

The results are shown in the following tables:

EXAMPLE 1.—POLYMER A

| Product                | Weight percent | Cu percent | Efficiency, Cu percent | CaO+MgO, percent | Efficiency CaO+MgO, percent |
|------------------------|----------------|------------|------------------------|------------------|-----------------------------|
| 1st concentrate.....   | 2.4            | 26.15      | 33.3                   | 4.40             | 0.7                         |
| 2nd concentrate.....   | 1.3            | 17.40      | 12.2                   | 6.23             | 0.5                         |
| 3rd concentrate.....   | 0.7            | 15.50      | 6.0                    | 7.13             | 0.3                         |
| Total concentrate..... | 4.4            | 21.80      | 51.5                   | 5.40             | 1.4                         |
| Waste.....             | 95.6           | 0.94       | 48.5                   | 15.37            | 98.6                        |
| Supply.....            | 100.0          | 1.85       | 100.0                  | 14.93            | 100.0                       |

EXAMPLE 2.—POLYMER B

| Product                | Weight percent | Cu percent | Efficiency, Cu percent | CaO+MgO, percent | Efficiency CaO+MgO, percent |
|------------------------|----------------|------------|------------------------|------------------|-----------------------------|
| 1st concentrate.....   | 1.6            | 29.40      | 25.3                   | 4.59             | 0.5                         |
| 2nd concentrate.....   | 1.4            | 20.25      | 15.2                   | 6.02             | 0.6                         |
| 3rd concentrate.....   | 0.8            | 17.10      | 6.0                    | 6.92             | 0.3                         |
| Total concentrate..... | 3.8            | 23.50      | 47.4                   | 5.55             | 1.4                         |
| Waste.....             | 96.2           | 1.02       | 52.6                   | 15.20            | 98.6                        |
| Supply.....            | 100.0          | 1.86       | 100.0                  | 14.83            | 100.0                       |

EXAMPLE 3.—POLYMER C

| Product                | Weight percent | Cu percent | Efficiency, Cu percent | CaO+MgO, percent | Efficiency CaO+MgO, percent |
|------------------------|----------------|------------|------------------------|------------------|-----------------------------|
| 1st concentrate.....   | 1.7            | 28.70      | 26.4                   | 4.34             | 0.5                         |
| 2nd concentrate.....   | 1.2            | 21.40      | 14.0                   | 5.30             | 0.4                         |
| 3rd concentrate.....   | 0.9            | 17.90      | 9.3                    | 6.34             | 0.4                         |
| Total concentrate..... | 3.8            | 24.30      | 49.7                   | 5.03             | 1.3                         |
| Waste.....             | 96.2           | 0.96       | 50.3                   | 15.20            | 98.7                        |
| Supply.....            | 100.0          | 1.88       | 100.0                  | 14.83            | 100.0                       |

A second series of examples (4 and 5) relates to the treatment of lead-bearing waste, rich in cerusite and having a calcareous gangue which are submitted in known manner to a sulfuration treatment. This waste was ground to 85 percent—200 mesh, in the presence of sodium silicate (100 grams per ton). It was then treated by sulfuration and flotation in a laboratory Denver cell. The consumption of reagents was as follows:

Sulfuration agent: 3.8 kg. of sodium hydrosulfide per ton of ore;

Collector: 160 grams of amyloxanthate of potassium per ton of ore;

Foaming agents: 30 grams of cresylic acid and 20 grams of Dowfroth 250 per ton of ore.

The results are shown in the following table:

| Product                | Weight percent | Pb percent | Efficiency, Pb percent |
|------------------------|----------------|------------|------------------------|
| 1st concentrate.....   | 7.9            | 52.02      | 48.5                   |
| 2nd concentrate.....   | 5.3            | 37.60      | 23.8                   |
| 3rd concentrate.....   | 3.3            | 18.51      | 7.3                    |
| Total concentrate..... | 16.5           | 40.62      | 79.6                   |
| Waste.....             | 83.5           | 2.06       | 20.4                   |
| Supply.....            | 100.0          | 8.42       | 100.0                  |

These results will be compared with those obtained in the two examples of application 5 and 6 which follow below; of methods and products according to the invention, which utilize respectively:

5 Example 4e: A gangue modifier D constituted by a modifier similar to the preceding modifying agents A, B and C, having a viscosity equal to 6 to 7 centipoises;

Example 5e: The gangue-modifying agent B of the previous example 2, the viscosity of which is 50 centipoises.

In the two examples 4 and 5, there have been added 780 grams of polymer per ton of ore, all the other conditions of sulfuration treatment being furthermore kept the same.

15 As clearly shown in all the examples given, the addition of a relatively small quantity of acrylic acid polymer has at all times a good effect on the efficiency and on the content of the concentrate.

EXAMPLE 4e.—POLYMER D

| Product                | Weight percent | Pb percent | Efficiency, Pb percent |
|------------------------|----------------|------------|------------------------|
| 1st concentrate.....   | 7.9            | 57.12      | 53.8                   |
| 2nd concentrate.....   | 3.2            | 42.34      | 16.2                   |
| 3rd concentrate.....   | 1.6            | 30.68      | 5.7                    |
| Total concentrate..... | 12.7           | 50.12      | 75.7                   |
| Waste.....             | 87.3           | 2.34       | 24.3                   |
| Supply.....            | 100.0          | 8.39       | 100.0                  |

EXAMPLE 5e.—POLYMER E

| Product                | Weight percent | Pb percent | Efficiency, Pb percent |
|------------------------|----------------|------------|------------------------|
| 1st concentrate.....   | 9.5            | 52.12      | 58.7                   |
| 2nd concentrate.....   | 5.1            | 33.95      | 20.5                   |
| 3rd concentrate.....   | 1.7            | 25.50      | 5.3                    |
| Total concentrate..... | 16.3           | 43.60      | 84.5                   |
| Waste.....             | 83.7           | 1.56       | 15.5                   |
| Supply.....            | 100.0          | 8.43       | 100.0                  |

75 It will be understood that the five examples given above are in no way limitative and that, without thereby departing from the scope of the invention, the latter may be applied on the

one hand to the treatment of all minerals of any kind having a calcareous and/or dolomitic gangue or the like and, on the other hand, the nature and the proportions of the modifying additives employed either alone or in mixtures may be modified in any suitable manner, in addition to the collector and foaming additives of the flotation process.

Instead of acrylic acid polymers, there could particularly be employed all equivalent products, such as linear anionic polymers, soluble in water, obtained by the hydrolysis of polynitriles, of polyesters or of copolymers having the same general characteristics (depending on the nature of the gangues, and also on the nature of the minerals or ores treated).

The modifying products may be added to the pulp during the course of flotation, or before flotation in a conditioning tank, or otherwise.

I claim:

1. In the treatment of minerals and ores with calcareous and dolomitic gangue by flotation separation of said gangue in an aqueous flotation medium, the improvement which comprises adding to said flotation medium at least one modifying agent acting on said gangue selected from the group of water-soluble polymers of acrylic acid corresponding to the general formula:



5 wherein R is H or  $\text{CH}_3$ , X is H or a cation from the group consisting of Na, Li, K,  $\text{NH}_4$  and organic bases imparting water solubility to the polymer, and n is an integer corresponding to the degree of polymerization represented by a Brookfield viscosity of as low as 6 and as high as 50 centipoises at 25°C.

10 2. Method according to claim 1 which the material being treated is the residue from a primary flotation of a copper ore.

3. Method according to claim 1 in which the material being treated is a lead-bearing waste.

15 4. Method according to claim 1 in which the ore is an oxidized ore.

5. Method according to claim 4 in which the gangue is dolomitic and sulfurating agent is present in the flotation medium.

20 6. Method according to claim 5 in which the ore is a copper ore.

7. Method according to claim 4 in which the ore is a lead ore and a sulfurating agent is present in the flotation medium.

25

30

35

40

45

50

55

60

65

70

75